

## UNITED STATES PATENT OFFICE.

GUILLAUME JUSTINE KROLL, OF LUXEMBURG, LUXEMBURG.

## PROCESS FOR THE PRODUCTION OF ALLOYS OF LEAD WITH ALKALINE EARTH METALS.

No Drawing. Application filed December 20, 1926, Serial No. 156,072, and in Germany December 29, 1925.

This invention relates to a process for the production of alloys of lead with alkaline earth metals.

As is well known it is possible to obtain 5 alloys of lead with the alkaline earth metals by heating lead with carbides of the alkaline earth metals or with mixtures forming such carbides. Owing to its high affinity for lead the alkaline earth metal is simply dissolved 10 out from the carbide, leaving the carbon. This solution process requires a temperature of about 1300° C., when the operation is carried out in graphite crucibles with access of air. At this temperature lead already possesses 15 a considerable vapour tension so that the workmen are exposed to the danger of poisoning by lead fumes. A further disadvantage of the above described process is that at the most, only 25% of the alkaline earth 20 metal contained in carbide is dissolved out and that the amount of lead run out only amounts at a maximum to 92% of the starting material.

Practical examination of this process has 25 moreover shown that it is impossible to carry it out as a continuous operation wherein the lead must be heated in graphite crucibles for a prolonged period at about 1300° C. After a short time the porous crucibles allow the 30 liquid highly heated lead to penetrate therethrough.

It has now been found that the aforesaid 35 disadvantages of the carbide process can be obviated by certain measures. In the first place it is important to decrease the temperature. A correct recognition of the reaction taking place during this solution process, has shown that it is above all necessary to exclude the oxygen and nitrogen of the air. At temperatures upwards of about 1100° C., these 40 gases have an extraordinarily energetic oxidizing and nitrating action upon the carbide which is covered by a protective layer which prevents penetration of the lead, with the result that the solution process gradually ceases.

If, however the carbide is heated together 45 with the lead in an atmosphere of hydrogen, the solution of the alkaline earth metal already actively commences at about 800° C. The carbide is much more completely used up and the yield in alloy is much better.

For example a mixture of 1000 grammes lead with 50 grammes calcium carbide which

had been heated for one hour at 800° C., with 55 constant stirring yielded an alloy containing 2.1% calcium. The yield amounted to about 75% of the calcium contained in the carbide and 97% of the lead employed.

The heating may also be effected in an atmosphere of other gases such as argon or even 60 carbon monoxide instead of in hydrogen, as long as such gases remain more or less inert towards carbide at the temperature range in question. It is moreover sufficient to evacuate 65 the reaction vessels or to close them airtight or, in addition, to tighten them with charcoal in the way usual when glowing copper. Any measure for excluding the oxygen or the nitrogen of the air leads to the desired 70 end, namely the reduction of the solution temperature.

It is only by means of the above described 75 measures that it has been possible to carry out the carbide process for the production of alloys of lead with alkaline earth metals on a practical scale.

The working temperatures used range 80 from 700° to a maximum of 1000° C., so that the employment of iron crucibles was 85 rendered possible. The using up of the carbide and the removal of the metal could be improved to such an extent that the production of intermediate products is inconsiderable. When employing electric furnaces for 85 heating the charge, considerable current economy was obtained.

I claim:

1. A process for the production of alloys 90 of lead with alkaline earth metals which comprises heating lead at a reacting temperature not exceeding 1100° C. with alkaline earth metal carbides in the absence of substances which form around the carbides a protective layer impenetrable by lead. 95

2. A process for the production of alloys 100 of lead with alkaline earth metals which comprises heating lead at a reacting temperature not exceeding 1100° C. with alkaline earth metal carbides in the absence of oxygen and nitrogen.

3. A process for the production of alloys 105 of lead with alkaline earth metals which comprises heating lead at a reacting temperature not exceeding 1100° C. with alkaline earth metal carbides in a closed container impermeable to air.

4. A process for the production of alloys

of lead with alkaline earth metals which comprises heating lead at a reacting temperature not exceeding 1100° C. with alkaline earth metal carbides in an evacuated closed 5 container.

5. A process for the production of alloys of lead with alkaline earth metals which comprises heating lead at a reacting temperature not exceeding 1100° C. with substances 10 adapted to form alkaline earth metal carbides, said heating being effected in the absence of substances which form around the carbides a protective layer impenetrable by lead.

15. 6. A process for the production of alloys of lead with alkaline earth metals which comprises heating lead at a reacting temperature not exceeding 1100° C. with substances adapted to form alkaline earth metal carbides, said heating being effected in the absence of oxygen and nitrogen.

7. A process for the production of alloys of lead with alkaline earth metals which comprises heating lead at a reacting temperature not exceeding 1100° C. with substances 25 adapted to form alkaline earth metal car-

bides, said heating being effected in a closed container impermeable to air.

8. A process for the production of alloys of lead with alkaline earth metals which 30 comprises heating lead at a reacting temperature not exceeding 1100° C. with substances adapted to form alkaline earth metal carbides, said heating being effected in an evacuated closed container.

35 9. A process for the production of alloys of lead with alkaline earth metals which comprises heating lead at about 700° C. to 1100° C. with alkaline earth metal carbides in the absence of substances which form 40 around the carbides a protective layer impenetrable by lead.

10. A process for the production of alloys of lead with alkaline earth metals which comprises heating lead at about 700° C. to 45 1100° C. with substances adapted to form alkaline earth metal carbides, said heating being effected in the absence of substances which form around the carbides a protective layer impenetrable by lead.

In testimony whereof I affix my signature.  
GUILLAUME JUSTINE KROLL.